

April 19, 1938.

E. R. POWELL

2,114,353

## METHOD OF MAKING A THERMAL INSULATING UNIT

Filed April 17, 1934



**INVENTOR**  
*Edward R. Powell.*

BY D. N. Halstead.  
ATTORNEY.

## UNITED STATES PATENT OFFICE

2,114,353

## METHOD OF MAKING A THERMAL INSULATING UNIT

Edward R. Powell, Alexandria, Ind., assignor to  
Johns-Manville Corporation, New York, N. Y.,  
a corporation of New York

Application April 17, 1934, Serial No. 720,979

1 Claim. (Cl. 154—28)

This invention relates to a thermal insulating unit and the method of making the same, and particularly to a unit adapted for use at temperatures below the dew-point of vapor in the surrounding atmosphere.

It is an object of this invention to provide a preformed heat insulating bat of mineral wool fibers which is durable and especially light, fluffy and springy in character, and which will expand 10 and snugly fill all portions of a casing, when compressed therein, and maintain its position indefinitely in the casing when anchored thereto without settling or crumbling of the fibers, thereby adapting it for uses in which it is subjected 15 to jarring and constant mechanical vibrations.

The invention is illustrated in the drawing in which,

Fig. 1 shows a side elevational view of a unit representing the preferred embodiment of the 20 invention, in part broken away for clearness of illustration;

Fig. 2 shows the casing material, in open form, to be shaped into the case shown in Fig. 1;

Fig. 3 shows a cross sectional view on line 3—3 of Fig. 1;

Fig. 4 shows a cross sectional view of the wall of the case;

Fig. 5 shows a side elevational view of a modification of the invention in which a filler bat is secured to the case by stitching, the structure being broken away in part for clearness of illustration;

Fig. 6 shows a cross sectional view on line 6—6 of Fig. 5; and

Fig. 7 shows a cross sectional view on line 7—7 of Fig. 5.

In the various figures like reference characters denote like parts.

There is shown a lightweight pad or bat 10, of 40 felted fibrous material, enclosed within a moisture-proof and draft-proof case 11. The felt is resilient and contacts with the case.

The case is relatively stiff and its walls include, suitably, composited sheets of plane and corrugated paper. Thus, the walls may include 45 the corrugated sheet 12, adhered to one or more facing sheets 13 of plane paper, to form either single-faced or double-faced corrugated board having dead air spaces for insulating effect. The 50 several sheets comprising the corrugated board may be composed by means of sodium silicate adhesive (not shown). Moisture-proofness of the case may be provided by means of a continuous layer 14 of asphalt disposed between the 55 outer facing sheet of the corrugated board and a finishing sheet 15 that may also be paper of plane surface. This asphalt is preferably of melting point of about 95° to 100° F., by the ball and ring method, and very sticky at room temperature.

The package may include an inside stiffening liner 21, such as corrugated cardboard faced on each side with paper of plane surface. The member 15 may consist of two sheets of kraft paper, with a layer of asphalt adhering the two sheets 5 together.

The fibrous pad 10 is secured, either continuously or at intervals, to the interior faces of the case, as by means of adhesive material 16.

Joints in the finished case are closed by means 10 of paper strips 17, adhered over the joints, in moisture-proof manner, as by means of adhesive 18 of asphalt or the like. The asphalt, used for this sealing, is preferably rigid at atmospheric temperature and of melting point of about 170° 15 to 240° F.

To make a tightly sealed, waterproof package, it is necessary also to seal the ends. This may be done by dipping the ends into some melted gum or pitch, adapted to provide waterproofness, and 20 covering the dipped portion with paper. The paper is brought over the side faces and edges a short distance, as shown at 23. Also tape may be used, either in pre cemented form or with separately applied adhesive.

In constructing units of the type illustrated in 25 Figs. 1—4, there is first provided a suitable preformed, resilient lightweight and fluffy pad of 30 felted fibers of mineral wool, of which slag wool and rock wool are two commercial types. Particularly satisfactory results have been obtained when the fibers used are rock wool. A pad of such fibers may be made by a process including melting an argillaceous limestone, allowing the molten material to fall, in a small stream, into a 35 very rapidly moving steam jet, to shred the molten material into fibers, allowing the fibers to collect in the bottom of a settling chamber, as, for example, on a conveyor belt, in a felt of desired thickness, then shaping the felt on the top 40 and sides, while still warm, by compression, and, finally, cutting the felt thus formed into pads of predetermined length and breadth.

A modification of the process is made for the 45 present purpose, in that a small proportion of a skeletonizing, waterproofing, and stiffening agent is sprayed upon the fibers, in such manner that, although used in very limited amount, the said agent is uniformly distributed, to produce a wool which is especially light, fluffy and resilient. 50 Thus, there may be used an agent that is resilient and springy at ordinary temperatures, adhesive, and chemically inert towards the fibers, as, for example, an agent of the type of rosin or an asphalt having a relatively high melting point.

Apparatus and methods that may be used, with the modifications specified herein, in blowing the 55 wool, and collecting the fibers into the preformed felt, are described in U. S. Patent 1,899,056, issued to E. R. Powell, on February 28, 1933.

The invention will be particularly illustrated by the example in which asphalt of the type described is the skeletonizing agent applied.

The asphalt may be sprayed into the settling chamber, at a position near the nozzle which shreds the molten rock into wool, the asphalt being either premixed with the shredding steam or supplied adjacent thereto, by means of a separate pipe. The proportion of asphalt may be 10 small, say, of the order of 1.5 to 8 parts by weight to 100 parts of fibers. After being cooled, the integrally felted product is resilient, that is, resistant to permanent distortion when compressed slightly for a short time, and springy and self-sustaining, although weighing, in a typical bat, only about 6 pounds to the cubic foot.

The higher the melting point of the asphalt used, the more harsh and springy the finished product becomes.

20 The felted fibers are compressed and shaped into a bat while warm, soft and spongy, and before the skeletonizing and spacing agent has completely hardened, thereby producing a bat of predetermined size and density in which the fibers 25 are not broken or mutilated.

There is provided, also, in form ready to be shaped into a case and to be adhered to the felt, corrugated paper board, cut, for example, as illustrated in Fig. 2. To adhere the felt and to aid 30 in maintaining it in place, the inside of the case is coated with a cementing material which may be applied in the spaced stripes 16. Adhesive here used is suitably miscible, when in fluid or plastic form, with the stiffening agent present in 35 the pad 10, so that when the pad 10 is brought into contact with the adhesive on the case, there is formed an integral union or structure of the stiffening agent and adhesive. Thus, there may be used a soft asphalt, when the spacing agent 40 in the fibers is soluble or miscible therein. In general, the adhesive may be similar chemically to the stiffening agent; for example, both may be bituminous. The adhesive is suitably somewhat tacky at atmospheric temperatures whereas 45 the stiffening agent present should be more rigid or resilient. A soft asphalt may be used in the stripes; a hard asphalt may be used as the stiffening agent, as stated.

After the adhesive has been applied to the corrugated book wrap or folder, as, for example, 50 as illustrated in Fig. 2, then the preformed felt 10 is pressed thereupon. The cardboard is then bent or folded at the positions indicated by the dotted lines and formed around the bat, to 55 enclose it on all sides. The resiliency of the thus compressed felt causes reaction against the cardboard and facilitates adherence in the striped areas and more even spacing of the fibers in the finished unit. In view of the fact that the pads 60 are integrally formed, it is not necessary to coat entirely the walls of the container with adhesive in order to prevent the pads from pulling apart and settling upon being subjected to subsequent jarring and mechanical vibrations. The joints 65 in the case thus formed are then coated with a waterproof adhesive 18, as, for example, molten asphalt of high melting type, and strips of paper 17 are applied over the coating of adhesive, to give complete, moisture-proof sealing of all joints 70 and corners in the case. In the preferred method of making, the pads are cut over-sized and compressed into the containers while still warm and

soft, after which they set to a satisfactory rigidity.

A unit so made contains the pad in approximately established position. Furthermore, the felt is of substantially uniform density and therefore the settling or collapse under the influence 5 of vibration is reduced to a minimum. Moisture cannot affect the interior of the unit, inasmuch as moisture is excluded therefrom and also because the fibers themselves are preferably moisture-proofed by the asphalt or similar water-impermeable skeletonizing agent. Furthermore, the article is draft-proof and not subject to transfer of heat by the passage of air currents inwardly through one face and outwardly through the other face.

The modification illustrated in Figs. 5-7 is useful for purposes in which evenness of spacing of the fibers of the degree obtainable in the structure illustrated in Figs. 1 to 3 is not necessary. In the modification there is used a pad of fibers 20 and a case of the type described. A departure from the structure previously described is made, however, in that the felt 24 is secured in position, by means of stitching 19, directly to the case. The felt may be stitched by a gang sewing machine with needles spaced 3 to 5 inches apart, for instance, or the felt may be stitched thus to a separate supporting element 21, say of corrugated cardboard, and the case then shaped around this element and the felt stitched thereto. To decrease still further the settling of the fibers in the pad, when the pad is in use, and stabilize the size, the stitched felt may be subjected, during assembly of the unit, to jarring or jolting, to establish in part the settling thereof, and a separate felt 20 then supplied to fill the space developed by the jarring and jolting and to occupy spaces developed by the stitching, as illustrated in Figs. 6 and 7. Thus, if the bat and supporting element are jarred edgewise the space left above 40 the upper edge of the felt would be filled by the additional felt.

Finally, the shape or closure of the case may be further established by staples 22 inserted at suitable positions, to secure together overlying 45 portions of the casing material.

Units of the type described that have been found particularly satisfactory in the insulation of electrical refrigerators have been made of the following approximate typical overall dimensions: 21 x 17½ x 2 inches. By far the greater part of the thickness of 2 inches in such a unit corresponds to the thickness of the pad 10 of fibrous material.

The details that have been given are for the 55 purpose of illustration, not restriction, and variations within the scope of the claim may be made without departing from the spirit of the invention.

What I claim is:

A method of making an insulating unit comprising converting molten material into mineral wool fibres, uniformly mixing with the hot fibres a binding or skeletonizing material which is a solid at normal temperatures, felting said fibres 65 and material into a coherent pad, shaping said pad, applying slight, uniformly distributed pressure to the pad, and confining the warm pad before the binder solidifies in a stiff, form-retaining casing.

EDWARD R. POWELL.